

## UNITED STATES PATENT OFFICE.

EDUARD HEBERLEIN, OF WATTWIL, SWITZERLAND.

## COTTON GOODS WITH LINENLIKE EFFECT AND PROCESS OF PRODUCING SAID EFFECT.

No Drawing.

Application filed June 30, 1922. Serial No. 572,032.

*To all whom it may concern:*

Be it known that I, EDUARD HEBERLEIN, a citizen of the Swiss Republic, and resident of Wattwil, Canton of St. Gall, Switzerland, 5 have invented certain new and useful Improvements in Cotton Goods with Linenlike Effect and Processes of Producing Said Effect, of which the following is a specification.

10 My invention relates to cotton goods with linenlike effect and process of producing said effect.

The objects of the invention are to produce cotton goods having permanent linenlike effects; that is to say, cotton goods, webs and yarns having the characteristics of linen, and a process or processes by which such goods may be made by the treatment of cotton with certain reagents or chemicals.

15 Further objects and advantages of the invention will more fully appear from the following description setting forth preferred examples of processing such goods, and the invention will be pointed out more 25 particularly in the appended claims.

When cotton is treated according to the process of United States Letters Patent No. 1,265,082, granted to me May 7, 1918, i. e., with caustic soda of the concentration used 30 in mercerization and at temperatures below 0° C., the cotton acquires a transparent appearance. Transparent effects are also produced by processing fine cotton goods according to the process of United States Letters Patent to Georges Heberlein, Nos. 35 1,144,655, 1,201,961 and 1,288,885.

While this production of permanent transparent effects by the treatment of thin cotton goods was known by said prior 40 patents, they did not teach the production of the linen-like effects. According to the present invention the coarse, thick cotton webs and the corresponding yarns which are not capable of being transformed into transparent webs and yarns, acquire when treated 45 according to the process of said United States Letters Patent No. 1,265,082, not a transparent appearance, but a completely novel effect. Such coarse cotton goods 50 (yarns and webs) are profoundly changed by this process. They acquire a certain lustrous effect and a certain resistance to change of character by washing, and also acquire a considerable increase of strength. 55 These new properties which such goods ac-

quire when processed according to this invention, constitute as a whole an effect very accurately resembling linen, which is quite different from the transparent effect taught by the aforesaid prior patents. In the usual 60 and well-known so-called linen finish produced on cotton webs there is merely produced a temporary sticking together of the fibers, and the effect is completely lost after the first washing.

65 The remarkable behavior of the cotton goods which could not have been prophesied by knowledge of said prior patents, may be explained by saying that although the chemical reactions on the individual cotton 70 fibers in fine and in coarse yarns are the same, the effect as a whole is entirely different, according to the constitution of the yarn or web. It is not possible to draw a sharp boundary between the transparent effect and the new linen effect. However, it 75 may be affirmed that yarns or webs made therefrom which are of the order of fineness of the English Nos. above 80 exhibit transparency or border on transparency, whereas 80 all coarser yarns, that is to say, those under No. 80, exhibit the typical linen effect. It is to be remarked that according to the quality of the spun cotton, and in the case of webs according to their thickness, the 85 dividing line between the linen effects on the one hand and the transparent effects on the other hand, may vary somewhat from the yarn number above given.

85 In my said Letters Patent No. 1,265,082 it 90 was pointed out that the said permanent transparent effect could be obtained if the cotton fabric was treated for a sufficient period with caustic alkali cooled below 0° C. and of such concentration as would mercerize the cotton at the ordinary temperature, that is to say, of at least 15 deg. Bé. 95 specific gravity. It is also pointed out in that patent that variations in the effect could be obtained by treating the material 100 under tension, or by allowing more or less shrinkage during treatment, and that enhanced transparency could be obtained by treating the fabric with concentrated sulfuric acid of over 50½° Bé, in addition to 105 the said treatment with cold caustic soda, and that the sulfuric acid could be used in a cold state and could be used either before or after the caustic soda treatment. It is 110 further pointed out in that patent that the

treatment of the goods with the said cold caustic soda as set forth in said patent, could be used to replace the mercerization treatments at ordinary temperature in the processes described in the other aforementioned patents.

It has also been found here in the production of linen effects that, as was the case in my said process for producing transparent effects according to Patent No. 1,265,082, variations in effect could be obtained accordingly as the textile material is under tension during the cold mercerization, or is allowed to shrink more or less. Enhanced linen effects may be achieved if the coarse textile material mercerized at low temperature is subjected to the action of a suitable concentrated mineral acid, i. e., such for example as concentrated sulfuric acid of over 50.5° Bé. specific gravity or sulfuric acid of a lesser strength at a low temperature, or, if the textile material is first treated with concentrated sulfuric acid of over 50.5° Bé. specific gravity, or sulfuric acid of a lesser strength at a low temperature, and then treated with the caustic soda at low temperature. The sulfuric acid may also be used at a low temperature, say for example around 0° C. in order that the duration of its action may be extended, particularly in the case of thick textile goods. The operation of cold mercerization in the place of mercerization at room temperature, in the sense of the said United States Letters Patent No. 1,288,885, may also be used; that is to say, the treatment with caustic soda at low temperature may occur once or several times in alternation with treatments of the acid. Finally, the usual mercerization at normal temperature may be combined with the cold mercerization in the sense of my co-pending application for Letters Patent Serial No. 520,264, so as to enhance the lustrous effect.

The said coarse cotton goods when processed according to my present invention acquire or are converted into goods having a typical true linen effect. The web or cloth when thus treated and as compared to the said goods before treatment, becomes harder, stiffer, has more of a sheen, and appears smoother and more glass-like, seems cooler to the touch and acquires greater tensile strength, all of which are characteristics of linen, and as contrasted with the softer and more fuzzy, uneven looking cotton goods which lack a hard cool touch and are weaker in tensile strength. The coarse threads or yarns are, according to the present process, correspondingly changed to take on this linen effect.

The linen effect produced by the said treatment may be further enhanced in its character or improved by subjecting the textile material after the chemical treatments, to mechanical finishing operations, such as

pressing and smoothing, which may be carried out to the desired degree by means of calenders, mangles or the like.

Obviously, the process is applicable not only to simple webs, but to embroideries, 70 knitted goods, fancy goods, and, generally, to all coarse cotton textiles.

The following examples illustrate the invention:

*Example 1.*

75

Boiled cotton yarn, of English yarn No. 2, is impregnated with caustic soda lye of 30° Baumé specific gravity at -10° C. for one minute, then stretched, washed, bleached and 80 dried.

*Example 2.*

Mako-twist (twist-thread made of Egyptian cotton) of English yarn No. 50/2-fold, 85 which has been bleached and mercerized under tension in normal manner, is impregnated with caustic soda lye of 28° Baumé specific gravity at -13° C., for one and a quarter minutes, then washed and dried. 90

*Example 3.*

Bleached cotton fabric having 21/21 threads per one-quarter French inch and of English yarn No. 30/30 is impregnated with 95 caustic soda lye of 30° Baumé specific gravity at -10° C. for one minute, then washed and dried.

*Example 4.*

100

Bleached cotton fabric having 19/17 threads per quarter French inch, and of English yarn No. 38/44, is impregnated with sulfuric acid of 52° Baumé specific gravity for 5 seconds, washed and then treated with 105 caustic soda lye of 27° Baumé specific gravity at -12° C. for two minutes, and finally washed and dried.

*Example 5.*

110

Thick (closely woven), bleached cotton fabric having 25/27 threads per one quarter French inch and of English yarn No. 48/50, is impregnated with caustic soda lye of 31° Baumé specific gravity at -10° C. for one 115 minute, then washed and then treated for 15 seconds with sulfuric acid of 54° Baumé specific gravity at -5° C. It is finally washed and dried.

*Example 6.*

120

Lye-washed cotton fabric having 12/12 threads per one quarter French inch, and of English yarn No. 12/12, is impregnated with caustic soda lye of 20° Baumé specific gravity at -5° C. for half a minute, and then washed; during 10 seconds it is then drawn through sulfuric acid of 51° Baumé specific gravity at +5° C., again washed and finally treated with caustic soda lye of 130

25° Baumé specific gravity at  $-10^{\circ}$  C. for  $\frac{3}{4}$  of a minute; it is then washed, bleached and dried.

*Example 7.*

- 5 Bleached cotton fabric having 16/16 threads per one quarter French inch and of English yarn No. 20/20, is treated with caustic soda lye of 32° Baumé specific gravity at 10  $-8^{\circ}$  C. for  $1\frac{1}{2}$  minute and then mercerized under tension in normal manner, washed and dried.

Having thus described my invention in accordance with various preferred illustrations of the manner in which the process may be practiced on various characters of goods, what I claim is:

1. Process for producing permanent linen-like effects in cotton goods, which comprises taking for treatment cotton goods (yarns and webs) constituted of threads whose fineness does not exceed English yarn No. 80, and treating such goods with caustic alkali of at least 15° Baumé, at a temperature below  $0^{\circ}$  C.

2. Process for producing permanent linen-like effects in cotton goods, which comprises taking for treatment cotton goods (yarns and webs) constituted of threads whose fineness does not exceed English yarn No. 80, treating such goods with caustic soda at low temperature, then stretching the goods and washing it.

3. Process for producing permanent linen-like effects in cotton goods, which comprises taking for treatment cotton goods (yarns and webs) constituted of threads whose fineness does not exceed English yarn No. 80, and subjecting the goods to a plurality of chemical treatments, one a treatment with caustic alkali at low temperature to chemically structurally change the fibers, and another a treatment with a different cellulose solubilizing reagent which will differently chemically structurally change the fibers to produce in conjunction with said other treatment, said linen-like effect.

4. Process for producing permanent linen-like effects in cotton goods, which comprises taking for treatment cotton goods (yarns and webs) constituted of threads whose fineness does not exceed English yarn No. 80, and subjecting the goods to a plurality of chemical treatments, one a treatment with caustic alkali at low temperature, and another a treatment with a suitable concentrated strong mineral acid to produce in conjunction with said caustic alkali treatment, said linen-like effect.

60 5. Process for producing permanent linen-like effects in cotton goods, which comprises taking for treatment cotton goods (yarns and webs) constituted of threads whose fineness does not exceed English yarn No. 80, and subjecting the goods to a plu-

rality of chemical treatments, one a treatment with caustic soda of at least 15° Baumé at a temperature below  $0^{\circ}$  C., and another a treatment with concentrated sulfuric acid.

6. Process for producing permanent linen-like effects in cotton goods, which comprises taking for treatment cotton goods (yarns and webs) constituted of threads whose fineness does not exceed English yarn No. 80, and subjecting the goods to a plurality of chemical treatments, one a treatment with caustic soda of at least 15° Baumé at a temperature below  $0^{\circ}$  C., and another a treatment with sulfuric acid above 50° Baumé, and washing the goods after said acid treatment.

7. Process for producing permanent linen-like effects in cotton goods, which comprises taking for treatment cotton goods (yarns and webs) constituted of threads whose fineness does not exceed English yarn No. 80, and subjecting the goods to a plurality of chemical treatments, one a treatment with caustic soda of at least 15° Baumé at a temperature below  $0^{\circ}$  C., and another a treatment with concentrated sulfuric acid, and washing the goods after each of said treatments.

8. Process for producing permanent linen-like effects in cotton goods, which comprises taking for treatment cotton goods (yarns and webs) constituted of threads whose fineness does not exceed English yarn No. 80, and subjecting the goods to a plurality of chemical treatments, one a treatment with caustic soda of at least 15° Baumé at a temperature below  $0^{\circ}$  C., and another a treatment with concentrated sulfuric acid, and stretching the goods while being acted upon by at least one of said reagents.

9. Process for producing permanent linen-like effects in cotton goods, which comprises taking for treatment cotton goods (yarns and webs) constituted of threads whose fineness does not exceed English yarn No. 80, and subjecting the goods to a plurality of chemical treatments, one a treatment with caustic soda of at least 15° Baumé at a temperature below  $0^{\circ}$  C., and another a treatment with concentrated sulfuric acid, stretching the goods after it has been acted upon by at least one of said reagents, and washing the goods after each of said treatments.

10. Process for producing permanent linen-like effects in cotton goods, which comprises taking for treatment cotton goods (yarns and webs) constituted of threads whose fineness does not exceed English yarn No. 80, and subjecting the goods to a plurality of chemical treatments, one a treatment with caustic alkali of at least 15° Baumé at a temperature below  $0^{\circ}$  C., and another a treatment with a suitable concen-

- trated strong mineral acid, and washing the goods after each of said treatments.
11. Process for producing permanent linen-like effects in cotton goods, which 5 comprises taking for treatment cotton goods (yarns and webs) constituted of threads whose fineness does not exceed English yarn No. 80, and subjecting the goods to a plurality of chemical treatments, one a treatment with caustic alkali of at least 15° Baumé at a temperature below 0° C., and another a treatment with sulfuric acid at 10 low temperature.
12. Process for producing permanent 15 linen-like effects in cotton goods, which comprises taking for treatment cotton goods (yarns and webs) constituted of threads whose fineness does not exceed English yarn No. 80, and subjecting the goods to a plurality of chemical treatments, one a treatment with caustic alkali at low temperature, and another a treatment with a suitable concentrated strong mineral acid to produce in conjunction with said caustic alkali treatment, said linen-like effect, applying said treatments alternately in such manner that at least one of said treatments takes place between two applications of the other treatment.
13. Process for producing permanent 20 linen-like effects in cotton goods, which comprises taking for treatment cotton goods (yarns and webs) constituted of threads whose fineness does not exceed English yarn No. 80, and subjecting the goods to a plurality of chemical treatments, one a treatment with caustic alkali of at least 15° Baumé at a temperature below 0° C., and another a treatment with concentrated sulfuric acid, applying said treatments alternately in such manner that at least one of said treatments takes place between two applications of the other treatment, and washing the goods after each acid treatment.
14. Process for producing permanent 25 linen-like effects in cotton goods, which comprises taking for treatment cotton goods (yarns and webs) constituted of threads whose fineness does not exceed English yarn No. 80, and subjecting the goods to a plurality of chemical treatments, one a treatment with caustic soda of at least 15° Baumé at a temperature below 0° C., and another a treatment with sulfuric acid of over 50° Baumé, applying said treatments alternately in such manner that at least one of said treatments takes place between two applications of the other treatment, and washing the goods after each treatment.
15. Process for producing permanent 30 linen-like effects in cotton goods, which comprises taking for treatment cotton goods (yarns and webs) constituted of threads whose fineness does not exceed English yarn No. 80, and subjecting the goods to a plurality of chemical treatments, one a treatment with caustic alkali of at least 15° Baumé at a temperature below 0° C., and another a treatment with concentrated sulfuric acid at low temperature, and a third a mercerization treatment at ordinary temperature.
16. Process for producing permanent 35 linen-like effects in cotton goods, which comprises taking for treatment cotton goods (yarns and webs) constituted of threads whose fineness does not exceed English yarn No. 80, and subjecting the goods to a plurality of chemical treatments, one a treatment with caustic alkali of at least 15° Baumé at a temperature below 0° C., another a treatment with sulfuric acid at low temperature, and a third a mercerizing treatment at ordinary temperature.
17. Process for producing permanent 40 linen-like effects in cotton goods, which comprises taking for treatment cotton goods (yarns and webs) constituted of threads whose fineness does not exceed English yarn No. 80, and treating such goods with caustic alkali of at least 15° Baumé, at a temperature below 0° C., and then subjecting the goods to at least one mechanical finishing operation.
18. Process for producing permanent 45 linen-like effects in cotton goods, which comprises taking for treatment cotton goods (yarns and webs) constituted of threads whose fineness does not exceed English yarn No. 80, and subjecting the goods to a plurality of chemical treatments, one a treatment with caustic soda of at least 15° Baumé, at a temperature below 0° C., and another a treatment with concentrated sulfuric acid, and then subjecting the goods to at least one mechanical finishing operation.
19. Cotton goods (yarns and webs) 50 constituted of threads whose fineness does not exceed English yarn No. 80, and having a permanent linen-like effect produced by chemical treatment of the goods, comprising a treatment with caustic alkali of at least 15° Baumé, at a temperature below 0° C.
20. Cotton goods (yarns and webs) 55 constituted of threads whose fineness does not exceed English yarn No. 80, and having a permanent linen-like effect produced by chemical treatment of the goods, one a treatment with caustic alkali at low temperature to chemically structurally change the fibers, and another a treatment with a different cellulose solubilizing reagent which will differently chemically structurally change the fibers to produce in conjunction with said other treatment, said linen-like effect.
21. Cotton goods (yarns and webs) 60 constituted of threads whose fineness does not exceed English yarn No. 80, and having a permanent linen-like effect produced by chemical treatment of the goods, one a treatment with caustic soda of at least 15°

- Baumé, at a temperature below 0° C., and another a treatment with concentrated sulfuric acid.
22. Cotton goods (yarns and webs) constituted of threads whose fineness does not exceed English yarn No. 80, and having a permanent linen-like effect produced by chemical treatment of the goods, one a treatment with caustic alkali of at least 15° Baumé, at a température below 0° C., and another a treatment with sulfuric acid at low temperature.
- 10 Baumé, at a temperature below 0° C., and another a treatment with concentrated sulfuric acid, and washing the goods after each of said treatments.
23. Cotton goods (yarns and webs) constituted of threads whose fineness does not exceed English yarn No. 80, and having a permanent linen-like effect produced by chemical treatment of the goods, one a treatment with caustic alkali of at least 15° Baumé, at a température below 0° C., and another a treatment with sulfuric acid at low temperature.

In testimony whereof I have signed my name to this specification.

EDUARD HEBERLEIN.